

# UNITED STATES PATENT OFFICE.

HARRY SPURRIER, OF DETROIT, MICHIGAN.

## PROCESS OF TREATING COKE.

1,007,153.

Specification of Letters Patent. Patented Oct. 31, 1911.

No Drawing.

Application filed March 20, 1911. Serial No. 615,560.

To all whom it may concern:

Be it known that I, HARRY SPURRIER, a subject of the King of Great Britain, and a resident of Detroit, in the county of Wayne and State of Michigan, have invented a new and useful Process for Treating Coke, of which the following is a specification:

Coke usually contains sulfur, principally in the form of sulfates and sulfids of iron and of calcium, etc. When used to smelt or remelt iron and other metals in blast furnaces, cupolas and other similar furnaces, absolute contact or intermingling occurs between the coke and the melted metal so that this sulfur unites with the melted metal for which it has great affinity. The presence of more than a trace of sulfur in iron is objectionable, and more than one-sixteenth of one per cent. is sufficient to render the iron useless for many purposes.

To prevent the sulfur in the coke from uniting with the iron, it is necessary to provide a substance with which it will more readily unite when the coke is burned. Some of the salts, hydrates, and oxides of the alkali metals, particularly the carbonates, are particularly adapted for this purpose. Sodium carbonate is preferred because it may be dissolved in the cheapest solvent, water, and the coke moistened therewith, the solution being sprinkled or poured over the coke, or the coke immersed in the solution. As a result, the alkali is carried by the water into the pores of the coke where it may react on the sulfur just as soon as the conditions become proper and before the sulfur can unite with the iron. The strength of the solution will depend upon the condition of the coke and the amount of sulfur therein, but it should be less than a saturated solution, and the amount of carbonate should be in excess of

that indicated as necessary by an analysis of the coke. The water is then permitted to evaporate, spontaneously or otherwise. When the coke thus treated is used for melting iron, a soda slag is formed which contains the sulfur formerly in the coke, and which, by analysis, has been found often to contain also a portion of the sulfur formerly united with the iron. The sulfur in the slag is, probably in the form of sodium sulfate and of sodium sulfid, but I am uncertain as to the exact conditions. While sodium carbonate is the cheapest and therefore preferred substance to be employed, sodium hydrate, and sodium oxid ( $Na_2O$ ) and similar compounds of potassium may be employed if desired.

Having now explained my process and its advantages, what I claim as my invention and desire to secure by Letters Patent is:

1. The process of treating coke by moistening with a solution of a carbonate of an alkali metal, substantially as described.
2. The process of treating coke by moistening with a solution of sodium carbonate, substantially as described.
3. The process of treating coke containing sulfur which consists in moistening the coke with a solution of sodium carbonate to such an extent that after the solvent has evaporated, the carbonate will be in excess of an amount sufficient to combine with the sulfur in the coke.

In testimony whereof I have subscribed this specification in the presence of two subscribing witnesses.

HARRY SPURRIER.

Witnesses:

EDWARD N. PAGELSEN,  
ELIZABETH M. BROWN.